

## UNITED STATES PATENT OFFICE

AYLMER H. MAUDE, CLARENCE J. RODMAN, AND CHARLES A. STYER, OF WILKINSBURG,  
AND WILLIAM C. WILHARM, OF EDGEWOOD, PENNSYLVANIA, ASSIGNORS TO WEST-  
INGHOUSE ELECTRIC & MANUFACTURING COMPANY, A CORPORATION OF PENN-  
SYLVANIA

## DEOXIDIZER

No Drawing.

Application filed December 21, 1923. Serial No. 682,097.

This invention relates to means for removing oxygen from atmospheres containing the same, more especially to the removal of the oxygen from the spaces above the oil in electrical apparatus such as transformers, circuit breakers, oil switches and the like.

In such electrical apparatus it is customary to place the transformer body, or the like, within a metal container or tank and to cover the same with a high grade insulating oil. A space is left above the oil level to permit expansion thereof under normal operating conditions, and there is usually provided means whereby communication is allowed to the outside air, in order that upon expansion or contraction of the oil, air may be forced out or drawn in, a phenomenon which is known as breathing.

Upon an arc forming in the oil, either accidentally or during the normal operation of the apparatus, combustible gases which mix with the air in the space above the oil, are produced, forming an explosive mixture. This mixture has, on different occasions, been ignited by arcs within the apparatus, causing explosions which damaged the same, and endangered the lives of station attendants or workmen. Furthermore, the oxygen in the air which is breathed by the transformer, gradually reacts with the oil, forming a sludge which is detrimental to the insulating properties thereof.

In order to prevent the detrimental effects of oxygen, it has been proposed to provide an inert atmosphere in the container. One of the means was to provide a material through which all the air necessary for the breathing of the transformer shall pass, the material being capable of absorbing the oxygen from the air, thus rendering the atmosphere above the oil inert and preventing the formation of explosive mixtures.

Our invention relates to materials of this character, it being among the objects thereof to provide a material which shall be effective in removing oxygen from atmospheres containing the same, which shall not deteriorate and which shall be reactive under all the normal operating conditions of the apparatus.

In practicing our invention, we provide a mixture of a metal with an electrolyte and a relatively small amount of water. We have found that in the presence of certain substances capable of producing ions in solution, certain metals, such as copper, are capable of forming oxidation products with the oxygen of the air. We have further found that the use of equivalent proportions of the metal and electrolyte gives the best results. This is probably owing to the formation of a double salt of the two materials, which facilitates the oxidation reaction thereof.

The action may be accelerated by the addition of finely divided catalytic material, such as activated carbon and also by the use of highly porous inert material upon which the active ingredients are deposited. If desired, we may utilize a combination of the said materials in our mixtures.

It has been found that a mixture of this character, although effective at ordinary temperatures, becomes less effective at extremely low temperatures (below  $-15^{\circ}$  C.) and may cease to function if such extreme temperatures are reached. To prevent the loss of activity at the low temperatures, an electrolyte such as calcium chloride which is capable of depressing the freezing point of the material may be added, and is, in itself, capable of causing the metal to remain reactive.

The addition of an electrolyte to depress the freezing point, however, is not essential when the apparatus is being operated at normal atmospheric temperatures, its addition only being requisite when the apparatus is being operated at abnormal atmospheric temperatures. For example, when calcium chloride is added, the composition is stable and reactive at temperatures as low as  $-35^{\circ}$  C. It will be understood that the addition of calcium chloride does not form a part of the present invention, as compositions including its use are described and claimed in copending application, Serial No. 682,098 to Ford et al. which is also assigned to the Westinghouse Electric & Manufacturing Company.

Specifically, we provide a mixture of copper and ammonium chloride in equimolecular proportions, and add thereto a small amount of water. Into this mixture there 5 may be incorporated in any suitable manner, an inert material such as kieselguhr, a catalyst such as activated carbon and a substance such as hydrated calcium chloride. The following mixture including calcium 10 chloride has been found very effective in deoxidizing atmospheres:

|                                      | Per cent |
|--------------------------------------|----------|
| Copper                               | 44.6     |
| Ammonium chloride                    | 36.2     |
| 15 Kieselguhr                        | 4.2      |
| Calcium chloride (6H <sub>2</sub> O) | 6.3      |
| Activated carbon                     | 4.3      |
| Water                                | 4.4      |

20 A method of preparation of the above mixture which has been found suitable, is as follows: Copper oxide scale is ground and then mixed with 10% of its weight of silica, preferably in the form of kieselguhr. The mixture is then reduced with a reducing 25 gas, such as natural gas or other reducing gas such as hydrogen to give a mixture of finely divided copper and kieselguhr. The material is sifted to obtain particles which pass through a 200-mesh sieve, and the remaining ingredients are added and 30 mixed in an inert atmosphere of nitrogen or carbon dioxide.

Our preferred mixture for normal operating 35 conditions is the same as that given above with the exception that the calcium chloride is omitted. This would render the proportions substantially as follows:

|                   | Per cent |
|-------------------|----------|
| 40 Copper         | 47.6     |
| Ammonium chloride | 38.6     |
| Kieselguhr        | 4.5      |
| Activated carbon  | 4.6      |
| Water             | 4.7      |

45

100.0

Activated carbon may be substituted in whole or in part for the kieselguhr catalyst or spacer material since one of the main 50 purposes of the catalyst is to act as a separator for preventing the chemically reactive mixture from packing, and for maintaining the reactive material in such condition that the gas may readily and completely combine 55 therewith.

The reactive mixture may be packed in a container much the same as kieselguhr itself would be. When gas is passed over the surface of the material and conducted there 60 through, the total effect is that the gas reacts completely with the uppermost layers of the mixture, resulting in a sharply defined plane of demarcation that extends entirely across the container between the dis 65 colored layer of exhausted material and the

active material. Upon continuing the passage of the gas, the layer of exhausted material is gradually extended in a uniform manner, always maintaining a marked plane of division between the exhausted and active 70 material.

The method of preparation of the latter modification is the same as the method used in the former. The finely ground copper scale is mixed with the desired amount of kieselguhr and reduced to the metallic state. After separating the coarse material, the remaining ingredients are added and mixed in an inert atmosphere.

This mixture is very effective for the purpose specified, in that the material does not deteriorate on standing, since there is no undesirable reaction taking place between the ingredients thereof. It is not affected by the humidity of the air and by ordinary 25 temperature changes, and is stable up to a temperature of about 120° C.

Although we have described our invention setting forth specific embodiments thereof, various changes may be made in the composition and the manner of making the same, within the scope of our invention. For instance, instead of ammonium chloride, other ammonium salts such as the sulphate, fluoride, or the like may be used. The inert material may be inorganic or organic, such as cork dust, sawdust, asbestos or other materials having the desired characteristics. The activated carbon may be omitted if desired, but there are indications that both the inert material and the activated carbon are effective in increasing the efficiency of the reaction. The carbon may be in any of its well-known forms, such as carbon black, coke dust, activated charcoal, or deflocculated 100 graphite. The proportions of the ingredients may be varied within wide ranges and still produce effective mixtures.

While copper has been specifically mentioned and is preferred as the oxidizable 110 metal which may be utilized, it will be understood that other oxidizable metals may be employed such as those disclosed in copending application, Serial No. 682,075, assigned to the Westinghouse Electric & Manufacturing Company, which has matured into Patent No. 1,652,496, dated December 13, 1927.

115 We claim as our invention:

1. A material for deoxidizing atmospheres comprising copper, an ammonium salt, kieselguhr and water.

2. A material for deoxidizing atmospheres comprising copper, ammonium chloride, kieselguhr and water, the copper and ammonium chloride being in substantially 125 equimolecular proportions.

3. A material for deoxidizing atmospheres comprising an oxidizable metal, an electrolyte and a catalyst, said electrolyte being 130

non-reactive with said metal in the absence of oxygen.

4. A material for deoxidizing atmospheres comprising an oxidizable metal, an electrolyte and carbon, said electrolyte being non-reactive with said metal in the absence of oxygen.

5. A material for deoxidizing atmospheres comprising an oxidizable metal, an electrolyte that is non-reactive with said metal in the absence of oxygen and activated carbon.

10 6. A material for deoxidizing atmospheres comprising an oxidizable metal, an electrolyte that is non-reactive with said metal in the absence of oxygen, a catalyzer and water.

15 7. A material for deoxidizing atmospheres comprising an oxidizable metal, an electrolyte that is non-reactive with said metal in the absence of oxygen, activated carbon and water.

20 8. A material for deoxidizing atmospheres comprising copper, a salt of ammonia, kieselguhr, activated carbon and water.

25 9. A material for deoxidizing gases capable of reacting with oxygen at normal atmospheric temperatures which comprises an oxidizable metal, an ammonium salt and water.

30 10. A material for deoxidizing gases capable of reacting with oxygen at normal atmospheric temperatures which comprises copper, an inert spacing material, an ammonium compound and water, said copper and alkali compound being in substantially equimolecular proportions.

40 11. A material for deoxidizing gases capable of reacting with oxygen at normal atmospheric temperatures which comprises a mixture of finely divided copper, a finely divided inert material and ammonium chloride.

45 12. A material for deoxidizing gases capable of reacting with oxygen at normal atmospheric temperatures comprising 40 to 60 parts of a finely divided oxidizable metal, a substantially equimolecular proportion of an ammonium compound, approximately 4 parts of finely divided inert material and water.

50 13. A material for deoxidizing gases capable of reacting with oxygen at normal atmospheric temperatures comprising 40 to 60 parts of finely divided copper, a substantially equimolecular proportion of an ammonium compound, approximately 4 parts of finely divided inert material and approximately 5 parts of water.

55 14. A material for deoxidizing atmospheres comprising copper, an ammonium salt, kieselguhr, activated carbon and water, the copper and chloride being in substantially equimolecular proportions.

60 15. A material for deoxidizing atmos-

pheres comprising copper, ammonium chloride, kieselguhr, activated carbon and water, the copper and chloride being in substantially equimolecular proportions and the kieselguhr and carbon being in minor proportions.

65 16. A material which comprises a metal oxidizable at temperatures below 120° C. and an electrolyte that is non-reactive with said metal in the absence of oxygen, said metal and electrolyte being chemically active toward each other in the presence of oxygen and toward atmospheres at normal atmospheric temperatures, whereby oxidizing gases in said atmospheres are reduced.

70 17. A material which comprises substantially equivalent proportions of a metal oxidizable at temperatures below 120° C. and an electrolyte, said metal and electrolyte being chemically active toward each other in the presence of oxygen and toward atmospheres at normal atmospheric temperatures, whereby oxidizing gases in said atmospheres are reduced.

75 18. A material which comprises water, a metal oxidizable at temperatures below 120° C. and an electrolyte that is non-reactive toward said metal in the absence of oxygen, said metal and electrolyte being chemically active toward each other in the presence of oxygen and toward atmospheres at normal atmospheric temperatures, whereby oxidizing gases in said atmospheres are reduced.

80 19. A material which comprises water, substantially equivalent proportions of a metal oxidizable at temperatures below 120° C. and an electrolyte that is non-reactive toward said metal in the absence of oxygen, said metal and electrolyte being chemically active toward each other in the presence of oxygen and toward atmospheres at normal atmospheric temperatures, whereby oxidizing gases in said atmospheres are reduced.

85 20. A material which comprises a metal oxidizable at temperatures below 120° C. and an ammonium salt, said metal and salt being chemically active toward each other and toward atmospheres at normal atmospheric temperatures, whereby oxidizing gases in said atmospheres are reduced.

90 21. A material which comprises substantially equivalent proportions of a metal oxidizable at temperatures below 120° C. and an ammonium halide salt, said metal and salt being chemically active toward each other and toward atmospheres at normal atmospheric temperatures, whereby oxidizing gases in said atmospheres are reduced.

95 22. A material which comprises water, a metal oxidizable at temperatures below 120° C. and an ammonium halide salt, said metal and salt being chemically active toward each other and toward atmospheres at normal atmospheric temperatures, whereby oxidizing gases in said atmospheres are reduced.

23. A material which comprises water, substantially equivalent proportions of a metal oxidizable at temperatures below 120° C. and an ammonium halide salt, said metal and salt being chemically active toward each other and toward atmospheres at normal atmospheric temperatures, whereby oxidizing gases in said atmospheres are reduced.

24. A material which comprises copper and an electrolyte that is non-reactive toward copper in the absence of oxygen, said copper and electrolyte being chemically active toward each other in the presence of oxygen and toward atmospheres at normal atmospheric temperatures, whereby oxidizing gases in said atmospheres are reduced.

25. A material which comprises substantially equivalent proportions of copper and an electrolyte that is non-reactive toward copper in the absence of oxygen, said copper and electrolyte being chemically active toward each other in the presence of oxygen and toward atmospheres at normal atmospheric temperatures, whereby oxidizing gases in said atmospheres are reduced.

26. A material which comprises water, copper and an electrolyte that is non-reactive toward copper in the absence of oxygen, said copper and electrolyte being chemically active toward each other in the presence of oxygen and toward atmospheres at normal atmospheric temperatures, whereby oxidizing gases in said atmospheres are reduced.

27. A material which comprises water, substantially equivalent proportions of copper and an electrolyte that is non-reactive toward copper in the absence of oxygen, said copper and electrolyte being chemically active toward each other in the presence of oxygen and toward atmospheres at normal atmospheric temperatures, whereby oxidizing gases in said atmospheres are reduced.

28. A material which comprises finely divided copper and an electrolyte that is non-reactive toward copper in the absence of oxygen, said copper and electrolyte being chemically active toward each other and toward atmospheres at normal atmospheric temperatures, whereby oxidizing gases in said atmospheres are reduced.

29. A material which comprises water, finely divided copper and an electrolyte that is non-reactive toward copper in the absence of oxygen, said copper and electrolyte being chemically active toward each other in the presence of oxygen and toward atmospheres at normal atmospheric temperatures, whereby oxidizing gases in said atmospheres are reduced.

30. A material which comprises water, copper and ammonium chloride, said material being chemically active toward atmospheres at normal atmospheric temperatures,

whereby oxidizing gases in said atmospheres are reduced.

31. A material which comprises water, copper and ammonium chloride, said copper and ammonium chloride being present in substantially equivalent proportions to form a complex salt, chemically active toward atmospheres at normal atmospheric temperatures, whereby oxidizing gases in said atmospheres are reduced.

32. A material which comprises water, finely divided copper and ammonium chloride, said material being chemically active toward atmospheres at normal atmospheric temperatures, whereby oxidizing gases in said atmospheres are reduced.

33. A material which comprises finely divided copper, ammonium chloride and water distributed throughout a mass of inactive spacing material, said material being chemically active toward atmospheres at normal atmospheric temperatures, whereby oxidizing gases in said atmospheres are reduced.

34. A material which comprises finely divided copper, ammonium chloride and water distributed throughout a mass of inactive spacing material, said copper and ammonium chloride being in substantially equivalent proportions, said material being chemically active toward atmospheres at normal atmospheric temperatures, whereby oxidizing gases in said atmospheres are reduced.

In testimony whereof, we have hereunto subscribed our names this 17th day of December, 1923.

AYLMER H. MAUDE.  
CLARENCE J. RODMAN.  
CHARLES A. STYER.  
WILLIAM C. WILHARM.

105

110

115

120

125

130